

April 14, 1936.

R. W. WILLIAMSON

2,037,294

LAMINATED MATERIAL

Original Filed Jan. 11, 1933



*Roger W. Williamson* Inventor

*By Wm. S. Hodges*

Attorney

## UNITED STATES PATENT OFFICE

2,037,294

## LAMINATED MATERIAL

Roger W. Williamson, Baltimore, Md.

Application January 11, 1933, Serial No. 651,235  
Renewed September 5, 1935

10 Claims. (Cl. 20—91)

This invention is a composite material primarily designed for wall or panel construction of the type in which the exposed area consists of a facing of wood veneer or other comparatively thin ornamental material usually to be applied to one side only of the preferred backing material. By means of such a composite construction it is possible to finish a room by applying the material sheet-like form directly to the studding, 5 omitting the usual plaster, thereby producing a wood-paneled room at low cost and with additional advantages, as will hereinafter appear.

Heretofore, attempts have been made to produce composite fireproof or incombustible wall 15 material, by attaching wood veneer or other sheet-like ornamental surfacing, to wood cores which have been treated to render them "fire-resistant". These attempted composite structures have failed to achieve commercial success 20 for various reasons, which will now be enumerated.

In the first place, the art of wood veneering involves a peculiar technique developed over a period of centuries. As is well known, wood 25 veneering facings have long been applied to wood cores, but the technique of the art makes it mandatory that the grain of the face and backing veneer must not run parallel with that of the core. Therefore, the veneer is usually applied 30 to the core in such manner that their respective grains are disposed at right angles to each other, so as to avoid twisting of the composite structure and cracking of the facing material. In fact, the best practice dictates that the core 35 be formed of ply board, i. e. a plurality of superposed veneer-like sheets firmly cemented together, and disposed with their respective grains in criss-cross relation. By such arrangement they attempt to neutralize strains and provide a 40 durable structure. The difficulties of obtaining the necessary equality of properties in two directions are such that those skilled in the art not only consider it advisable to use the same type of veneer for facing and backing, but even consider it necessary that the facing and backing 45 be both slice cut, both rotary cut or both saw cut. Certainly, omission of the backing veneer could not be even considered.

In the second place, walls or panels constructed 50 of cores which have been rendered fire-resistant by the commonly known impregnation methods, and wood veneers bound thereto, have been found impracticable in use, and are avoided by the architects wherever possible. This is because the material used in the so-called "fire-proofing", and the finishing materials used on 55 the wall or panels, in course of time react to cause change of color and appearance of spots over the areas. In addition to this, wood which 60 has been processed to render it fire-resistant is

difficult to mill because the processing material contained therein quickly ruins the cutting edges of all knives and other cutting tools, thereby greatly increasing the cost of installation as well.

Attempts have been made to attach such ornamental surfacing to slabs or sheets constructed of the so-called "fire-proof" materials, in which asbestos is normally included as an ingredient, because of its fire-resistant characteristics.

In the manufacture of fire-resistant wall material of the asbestos type, it is common to use either gypsum or hydraulic cement as a binder. The gypsum base is commercially impracticable for use as a core for veneer, because it lacks the necessary tensile strength to prevent the veneer 10 from stripping from the surface of the core, and it is so soft that it breaks away at the edges. When hydraulic cement is employed as the binder, the proportions of cement commonly employed are so high with respect to the other 15 constituents, as to provide a very hard more or less brittle board which is friable at the edges. In fact, the material is so hard and brittle that it cannot be penetrated by nails or similar fastening devices, for the purpose of securing the 20 sheets to the wall studding. Therefore, holes must be bored therein for the passage of screws 25 or nails, with the result that the boards frequently fracture during the boring operation, and in practice will also fracture in the vicinity of said 30 nail holes when the holding strain of the nail is brought to bear upon the slab. In addition to the foregoing, wall boards of this type will crack under intense heat, thereby rendering it more or less unstable.

When the mix is modified by adding another 35 ingredient, such as vermiculite or any of its equivalents, the board will not be so brittle, but in that modified state it will lack the tensile strength necessary to hold the veneer against 40 the stripping tendency described as existing when gypsum board is used.

However, a board of the so-called "asbestos" type, unlike the non-homogeneous wood-core, with its widely different strength properties in 45 the various directions relative to the grain, does not ordinarily require a balancing backing veneer when faced with an ornamental veneer. In special instances it may be preferred, and where 50 its use is such that both surfaces of the board can be seen, it is necessary for appearance.

Another important factor is that the commonly known commercial adhesives are not capable of effecting a permanent bond between the refractory or asbestos cores and the veneer or other 55 facing. For instance, cores of this type have depressions in some portions of the surface areas, and it is therefore necessary to even the surface to which the facing is to be attached, said evening being accomplished by sanding or otherwise, 60

in order to insure that the core and the veneer and the adhesive are all evenly contacting under the pressure developed by the press. Also, adhesives with acid characteristics have been tried, 5 and the acid of these types of adhesive react in an objectionable manner upon the alkaline characteristics of the core material, so that the strength of the adhesive is impaired and there is a liability that the veneer facing will be stained 10 and spotted, and the bond weakened or destroyed.

Bearing in mind the various objections heretofore encountered in the art, one of the objects 15 of the present invention is to provide a composite structure comprising a refractory core of the type which includes asbestos as one ingredient and hydraulic or Portland cement as a binder and having attached thereto a facing of wood veneer or other sheet-like ornamental material. A further object is to provide a heat-resistant composite 20 structure, in which an incombustible core of low thermal conductivity may be substituted for the fire-resistant wood now in common use in fireproof building construction. A further object is to produce a refractory core member of 25 the fire-resistant type which includes asbestos as one of its fire-resistant constituents and hydraulic or Portland cement as a binder, which core-member may be readily penetrated by nails, screws and other fastening devices and which will 30 not crack under high heat. A further object is to provide a composite structure comprising a core composed of infusible non-metallic silicates, provided with a veneer or other similar facing attached thereto, by means of an adhesive which 35 will fill depressions in the core surface and which will provide an effective bond without the necessity of sanding or otherwise smoothing the surfaces of the core. A further object is to provide a composite structure comprising a core member 40 consisting of non-combustible plastic silicates and an ornamental surface attached by means of an adhesive containing an ingredient which neutralizes any degree of acidity of the wood, as well as any degree of acidity in the finishing materials. A further object is to provide a composite 45 structure of the character mentioned in which the adhesive contains rubber in a form which is normally held in solution but capable of congealing after being applied to the surfaces to be bonded, thereby providing a perfect bond between the materials, and which at the same time interposes a moisture-resistant and acid neutralizing bond between the surface material and the core, and also a resilient bond between the 50 core and the surface material, which bond furthermore possesses sound deadening characteristics.

The invention will be hereinafter fully set forth and particularly pointed out in the claims.

60 In the accompanying drawing:—

The figure is a longitudinal sectional view of a sheet-like composite board constructed in accordance with the invention. In this connection, it is to be understood that the structure is shown 65 in more or less diagrammatic form for illustrative purposes only, and without intending to limit the invention, because it is obvious that the material may be in block or any other geometrical form.

70 Referring to the drawing, 10 designates the non-combustible fire-resistant core, 11 the ornamental facing, which may be wood veneer or any other ornamental surface materials, such as those of the cellulose type, the core and the facing being 75 united by an adhesive 12. If desired, the

rear surface of the core 10 may be likewise veneered or be painted with a suitable substance 13 to render it more moisture resistant, for which purpose any material which may be applied by means of a solvent carrier may be used, provided 5 that it has the desired body, although it is preferred to employ aluminum paint for this purpose.

The core 10 is constructed of a mixture of infusible non-metallic silicates including a silicate binder and a silicate ingredient which so tempers and toughens the sheet as to render it crack-resistant, and fire-resistant without destroying its tensile strength. A preferred material is described and claimed in a concurrently filed application for patent by Roger W. Williamson and Guy Leonard, Serial No. 651,236, and no claim is here made to the core per se.

As described in said application the material constituting the core 10 comprises a mixture 20 which includes asbestos, a micaceous material such as vermiculite, or its equivalent, kaolin and hydraulic or Portland cement as a binder. Such a core is approximately crack and fracture proof, under all conditions, is easily cut and fastened 25 to supporting material. If it is not desired to take advantage of these characteristics, any other mixture of the infusible non-metallic silicate type may be substituted as the core. It will be noted that the asbestos, vermiculite and kaolin 30 are all infusible non-metallic silicates cemented by an infusible, non-metallic silicate binder, i. e. hydraulic or Portland cement. It is also important to observe that the ingredients of which the core is constructed are alkaline in character. 35

The surfacing 11 and the core 10 are united by an adhesive in which latex held in suspension, is included as a constituent together with other adhesive materials carried by a solvent. This adhesive has the physical characteristic that it 40 will fill the valleys or pits in the rough surface of the core material, and will produce a strong bond under any temperature conditions which will permit the rubber to congeal, so that preliminary sanding of the surfaces is unnecessary. Chemically it is alkaline, and does not react with the alkalinity of the non-metallic silicates to injure the bond, and at the same time it neutralizes any acids in the wood which otherwise would react on the alkaline core. An adhesive which has 45 been found suitable for this purpose is disclosed in a copending application filed by Frank H. Shoals, concurrently herewith Serial No. 651,229.

The cores 10 may be made in any desired shape, usually in flat sheet-like form of predetermined dimensions. To produce the composite structure of the present invention, the more or less rough surface of the core to be faced is first covered with a coating of the adhesive. The facing material is then superposed upon the core and subjected to moderate heat and pressure. The coating 13 may then be applied, or if desired it may be applied prior to the attaching of the facing.

The advantages of the invention will be readily understood by those skilled in the art to which it belongs. For instance, it will be noted that the adhesive possesses the characteristic of not only effectively binding the parts together, but also prevents weakening of the bond, as well as staining or spotting of the facing material by neutralizing any acid which may be present therein. A further advantage is that the veneer or other surfacing is applied to a core material which requires no cross-bonding layers or 70 75 80 85 90 95

backing veneer, and which may be penetrated by nails, so that it may be readily secured to wall stanchions or other supports, so that neat and clean fitting of the material in installation is possible. Another important advantage is that by constructing the core of infusible non-metallic silicates, the expense of installation of a composite material which may be utilized for ornamental interior walls where fireproof conditions may be desired, is greatly reduced because a much cheaper substitute is provided for the ordinary fire-resistant treated woods now commonly employed. At the same time a composite structure is provided which avoids the objections inherent to attempts to provide veneer surfaces to woods which have been treated with fire-resistant materials. An outstanding advantage is the providing of a material which, in addition to its fireproof quality, is sound-absorbing and of low thermal conductivity. As it is to be applied directly to the studding, plaster may be eliminated, and the finished wall be at once wood paneled. Heretofore, the effect of a wood-paneled room had to be secured at an additional cost to plastering, or some other wall-forming material. Also, in the prior usage of so-called wall boards considerable difficulty has been experienced because of their pulling apart at the joints. This trouble is fully discussed in "Wood Construction", the published findings of the National Committee on Wood Utilization published in 1929 (pages 285 and 286). Preferred joint constructions for strength and appearance have been developed and are disclosed and claimed in a concurrently filed application for patent by William T. Hormes, and no claim is here made for such joint construction.

Having thus explained the nature of the invention and described an operative manner of constructing and using the same, although without attempting to set forth all of the forms in which it may be made, or all of the forms of its use, what is claimed is:—

1. A laminated material consisting of a non-combustible rigid core comprising a mixture of asbestos, a foliated micaceous material, a hydraulic cement binder and a hydrous aluminum silicate tempering agent of the kaolin group, and a thin veneer-like facing adhering to one surface of said core.

2. A laminated material consisting of a rigid unfired non-friable, substantially hard and tough sheet-like refractory body comprising a mixture of hydraulic cement binder, asbestos, a foliated micaceous material and a tempering agent consisting of a hydrous aluminum silicate of the kaolin group, the proportion of the tempering agent with respect to the total mixture being such that said body is readily workable with edge tools and penetrable by sharp metal anchoring devices without danger of body fracture, and a thin veneer-like facing adhering to the surface of said core.

3. A laminated material consisting of a non-combustible rigid core comprising a hydraulic cement binder, asbestos, a foliated micaceous material and a hydrous aluminum silicate tempering agent of the kaolin group, said core having an alkaline reaction, a veneer-like facing covering a surface of said core, an interposed adhesive of alkaline reaction uniting the facing and the core, said adhesive including a substance which protects the alkalinity of said core, and a moisture-resistant coating on the other face of said core.

4. A laminated material consisting of a non-combustible rigid core comprising a mixture of a hydraulic cement binder, asbestos, a foliated micaceous material and a hydrous aluminum silicate tempering agent of the kaolin group, a veneer-like facing for said core, and an interposed adhesive of alkaline reaction uniting the facing and the core, said adhesive including a substance which protects the alkalinity of said core. 5

5. A laminated material consisting of a non-combustible rigid core comprising a mixture of a hydraulic cement binder, asbestos, a foliated micaceous material and a hydrous aluminum silicate tempering agent of the kaolin group, and an adhesive interposed between said core and said facing and possessing the characteristic of developing latent adhesive qualities upon the application of heat. 10 15

6. A laminated material consisting of a non-combustible rigid core comprising a mixture of a hydraulic cement binder, asbestos, a foliated micaceous material and a hydrous aluminum silicate tempering agent of the kaolin group, and an alkaline adhesive interposed between and uniting the facing and said core, said adhesive including 20 25 a rubber constituent.

7. A laminated material consisting of a non-combustible rigid core possessing low thermal conductivity, said core comprising a mixture of a hydraulic cement binder, asbestos, a foliated 30 micaceous material and a hydrous aluminum silicate tempering agent of the kaolin group, a wood veneer-facing for said core, and an adhesive bond between said core and the facing.

8. A laminated material consisting of a non-combustible unfired rigid core comprising a mixture of a hydraulic cement binder, asbestos, a foliated micaceous material and a hydrous aluminum silicate tempering agent of the kaolin group, said core being readily workable with edge tools 40 and penetrable by sharp metal anchoring devices without danger of body fracture, a wood veneer facing for the core, and an adhesive interposed between the facing and the core, said adhesive containing a resilient bonding material. 45

9. A laminated material consisting of a refractory unfired rigid core comprising a mixture of a hydraulic cement binder, asbestos, a foliated micaceous material and a hydrous aluminum silicate tempering agent of the kaolin group, said core having an alkaline reaction and having inherent surface depressions therein, a veneer-like facing for said core, and an adhesive uniting said facing to the core, said adhesive containing a resilient material capable of filling said surface 50 depressions in such manner as to provide an adhesive-coated surface coextensive with the total area of the core.

10. A laminated material consisting of a refractory unfired rigid core comprising a mixture of a hydraulic cement binder, asbestos, a foliated micaceous material and a hydrous aluminum silicate tempering agent of the kaolin group, said core having an alkaline reaction and having inherent surface depressions therein, a veneer-like 60 facing for said core, and an adhesive uniting said facing to the core, said adhesive containing an ingredient capable of neutralizing the inherent acidity of the facing, and also containing an ingredient capable of filling said depressions in such 65 manner that a level adhesive-coated surface is provided coextensive with the full area of the core surface. 70

ROGER W. WILLIAMSON.